

# UNITED STATES PATENT OFFICE.

ROBERT ABBOTT HADFIELD, OF SHEFFIELD, ENGLAND.

## PROCESS FOR IMPROVING THE MAGNETIC QUALITIES OF A MAGNETIC BODY.

1,122,385.

Specification of Letters Patent.

Patented Dec. 29, 1914.

No Drawing. Application filed March 21, 1907, Serial No. 363,657. Renewed May 26, 1914. Serial No. 841,143.

To all whom it may concern:

Be it known that I, ROBERT ABBOTT HADFIELD, a subject of the King of Great Britain, of Sheffield, England, have invented a certain new and useful Improvement in Processes for Improving the Magnetic Qualities of a Magnetic Body, of which the following is a specification.

The invention is a process for improving certain magnetic qualities of a magnetic body, and more especially of alloys of iron and silicon, or iron-silicon and aluminium, or iron-silicon and manganese, in order to increase the magnetic permeability and electric resistance and lower the hysteresis action of the said body; and thus to adapt it for use in ballast-coils, transformer-plates and like electrical apparatus, where the reduction of magnetic and electric losses to the lowest possible degree is of great importance.

In carrying my process into effect, I first heat the body to a relatively high temperature below its melting point and say between 900° and 1000° centigrade. I then cool it rapidly. I then reheat the body to substantially the same temperature before mentioned and finally cause or allow it to cool slowly. By this process I attain the desirable result before mentioned.

Cooling rapidly, as herein referred to, means cooling at such a rate as that the changes effected by raising the material to the definite temperature stated are retained substantially unaltered.

Cooling slowly, as herein referred to, means cooling at such a rate as to permit the slow rearrangement of the molecules with reference to one another so that the condi-

tion of strain or hardness is removed and the material becomes soft, often accompanied by a more uniform distribution of the elements throughout the mass.

I claim:

1. The herein described process of reducing the total magnetic and electric loss in an iron silicon, aluminium, manganese alloy, which consists in first heating said alloy to a high temperature, below its melting point, then cooling said alloy rapidly, then reheating said alloy to substantially the same high temperature as before, and then cooling said alloy slowly.

2. The process of reducing the total magnetic and electric loss in an alloy containing iron and silicon, which consists in heating the alloy to a temperature ranging from about 900° C. to about 1000° C., then cooling said alloy rapidly, then reheating said alloy to substantially the same temperature as before, and then cooling said alloy slowly.

3. The herein described process of reducing the total magnetic and electric loss in an iron alloy, which consists in heating said alloy to a relatively high temperature below its melting point, then cooling the alloy rapidly so that the changes effected by heating the material to the high temperature stated are retained substantially unaltered, then reheating said alloy to substantially the same temperature as before and then cooling said alloy slowly.

In testimony whereof I have signed my name hereto in the presence of two witnesses.

ROBERT ABBOTT HADFIELD.

Witnesses:

WILLIAM CROSS,  
JOHN WM. CRAWLEY.